

May 3, 1927.

1,627,010

W. B. CAMPBELL

FREENESS TESTER FOR PULP

Filed June 21, 1926



INVENTOR

WILLIAM BOYD CAMPBELL

BY *Fetherstonhaugh Co*  
ATTORNEYS

Patented May 3, 1927.

1,627,010

# UNITED STATES PATENT OFFICE.

WILLIAM BOYD CAMPBELL, OF MONTREAL, QUEBEC, CANADA.

## FREENESS TESTER FOR PULP.

Application filed June 21, 1926. Serial No. 117,546.

This invention relates to new and useful improvements in the method of and apparatus for measuring the resistance offered to the flow of water through a bed of granular or fibrous material, and the object of the invention is to provide a simple and efficient means for measuring the resistance aforementioned, without the necessity for timing the flow of water or of measuring the temperature at which the test is made.

The device is particularly adapted for testing paper pulp during the course of manufacture, and is known in the art as a freeness tester.

From experiments on the mechanics of freeness testers of the type at present in use, it is evident that the freeness measured is really an indirect measure of the resistance offered by pulp to the flow of water through it, the pulp being in the condition in which it is found when it is deposited on a screen from a dilute suspension. The figures given by any of the testers at present in use, do not bear a direct relationship to this resistance since it involves several factors inherent in the particular tester used.

One of the outstanding advantages of the freeness tester of the type at present in use, is that there is no necessity for making measurement of time, but it has several disadvantages, one of which is its sensitivity to the temperature at which the determination is made. Another disadvantage is the comparatively large effect of small variations in the screen plate of the drainage chamber. A still further disadvantage is the variation in the freeness found if the time taken between starting the drainage and pouring the stock into the chamber is varied.

In my invention the apparatus used avoids the aforementioned disadvantages, while it retains the advantage of avoiding the necessity of timing the flow.

In the drawing which illustrates in diagrammatic form an apparatus suitable for testing the freeness of pulp by my improved method, 1 designates a constant level flow box, supplied by a stream of water through the side connection 2. This water flows in part through a short length of capillary tubing 3, and the overflow goes to waste through an overflow pipe 4. The head of water being constant, the flow of water through the capillary tube is proportional to the fluidity of the water. The lower part

of the tester consists of a long graduated transparent tube 5, which widens out at its lower end to a much larger diameter 6. A screen plate 7 having openings 8, sufficiently small to hold back substantially all of any pulp sample under test, is placed within the larger portion 6 of the tube and across the opening thereof. Just below the point 9 where the tube broadens out, a baffle 10 is placed to break up the stream line of flow through the narrow portion of the tube 5, and allow it to distribute over the larger area of the screen 7.

The operation of the device is as follows. A diluted sample of pulp of known dry weight, is poured into the upper end 11 of the tube 5, said upper end being funnel-shaped to facilitate this operation. As the dilute pulp flows down through the tube, the water drains from it through the screen plate and a sheet or mat of pulp is deposited on the plate. The pulp is thus deposited in the same manner as it is on a paper machine wire. Water is meanwhile flowing in at a constant rate through capillary tube and this water must pass through the pulp accumulated on the screen plate before passing out. When the pulp is all in the mat, a stable equilibrium will be established, so that there will be a head of water in the tube 5 just sufficient to cause as much water to flow out through the pulp mat as comes in through the capillary tube. At any one temperature the viscosity of the water is constant and there will therefore be a definite flow of water through the pulp. The pulp is spread over a definite area so that the resistance it offers to the definite flow is proportional to its "slowness" and its amount. The amount of the pulp is known from other determinations of consistency. The resistance offered is read off from the graduated tube at equilibrium. The flow is known from previous calibration of the instrument.

From these various factors the slowness of the pulp can be calculated in centimeter, gram, second units as offering a resistance of so many centimeters of water head per gram of pulp per square centimeter to a flow of one cubic centimeter per second. If it is desired to use freeness as a measure rather than slowness the reciprocal of the foregoing may be taken.

It is obvious that the test avoids the necessity of time measurements. How the disadvantages mentioned above are avoided

2  
may require some explanation. In the testers at present in use the temperature affects the test since it affects the viscosity of the water on which the rate of flow through the 5 pulp depends. Viscosity has practically no effect on turbulent flow or hydraulic flow, but it has a large effect on stream line flow, such as takes place through the pulp mat. In this tester herein disclosed the same effect 10 will take place i. e. the flow through the pulp will be more rapid as the viscosity is decreased through rise in temperature but so far as the resistance reading is concerned this effect is exactly balanced by the similar 15 effect on the flow through the capillary tube through which the flow is of the stream line type. The effect of variations in the screen plate is eliminated for all practical purposes since its resistance is an extremely small part 20 of the total resistance. This is not the case in the usual type of tester at present in use, particularly at the start of the flow which is the most important time. Since all the 25 pulp is on the screen plate, the time of settling ceases to have any influence.

The amount of flow can be set for any capillary used by regulating the head under which it operated, so that even if various sizes of capillaries are used, they will all 30 give the same result if the heads under which they operate are appropriately chosen.

In addition to avoiding these various difficulties, found in the usual type of tester, the tester herein disclosed has the advantage of 35 giving its results in absolute terms such as can be used in connection with sheet formation on the wire of a paper making machine. Very little difficulty would be encountered in making this device a recording instrument provided a reliable consistency regulator were available.

Having thus described my invention, what I claim is:—

1. An apparatus for measuring the 45 resistance offered to a flow of water through

a porous mat of material, comprising a graduated tube closed at its lower end by a screen plate to support the mat of material, and a device for feeding water to the tube at a fixed rate of flow sufficient to cause the 50 water to rise in the tube so as to register with the graduations thereon.

2. An apparatus for measuring the resistance offered to a flow of water through a porous mat of material, comprising a graduated tube expanded at its lower end, a screen plate supported in said end and upon which the material under test rests, and a constant level feed tank having a capillary tube depending from its lower end, the tube being 55 above the graduated tube and adapted to discharge thereinto.

3. An apparatus for measuring the resistance offered to a flow of water through a mat of pulp, comprising a graduated tube 65 expanded at its lower end, a screen plate secured to said end and covering the opening therefrom, means within the end above the screen plate to distribute pulp passing through the tube, evenly over the screen plate, a constant level water feed supply chamber having a capillary tube depending therefrom, and positioned over the graduated tube so as to discharge thereinto.

4. A method of measuring the resistance 75 offered by a mat of pulp to the passage of water therethrough, consisting of pouring a sample of diluted pulp through a vertical tube the lower end of which is closed by a screen plate over which the pulp becomes 80 distributed, passing water through the tube and the distributed pulp at a fixed rate of flow such that the water level will rise into the tube and finally reach a constant level 85 therein, and measuring the height of said constant level.

In witness whereof I have hereunto set my hand.

W. BOYD CAMPBELL.